

## UNITED STATES PATENT OFFICE.

HORACE RUSSELL McILHENNEY, OF RAHWAY, NEW JERSEY, ASSIGNOR TO VULCAN DETINNING COMPANY, OF SEWAREN, NEW JERSEY, A CORPORATION OF NEW JERSEY.

## ELECTRODEPOSITION OF TIN.

No Drawing.

Application filed April 14, 1926. Serial No. 101,921.

This invention relates to the electrodeposition of tin and has for its object an improvement in the electrodeposition of the tin.

Tin is electrodeposited by passing a direct current of electricity through an appropriate electrolyte such as a solution of a tin salt or compound. The electric current passes from one pole or electrode called the anode 10 through the electrolyte to the other pole or electrode called the cathode. As soon as this flow of electric current starts, all the anions in the solution begin to move toward the anode, while all the cations begin to move toward the cathode. In the case of a tin electrolyte, the metallic tin ions comprise at least 15 part of the cations, and in the course of the electrodeposition they are deposited as metallic tin in the cathode. The anions, and in the case of certain electrolytes some of the 20 cations, may escape as gas, or may be deposited on one of the electrodes in some form or other, or may react with the electrolyte to form new compounds that remain in the 25 electrolyte.

Various salts and compounds of tin may be used in preparing the tin electrolyte or electroplating bath. Thus, in commercial practice an aqueous solution of tin chloride 30 (stannous chloride) or an aqueous solution of sodium stannate are frequently used as electrolytes. As a direct current is passed through such an electrolyte, the metallic tin deposits on the cathode and the chlorine ions 35 or sodium ions, as the case may be, react with the water of the electrolyte to form hydrochloric acid or sodium hydroxide, respectively. Thus the tin content of the electrolyte is lowered and substances are formed 40 in the electrolyte which may be harmful to the proper deposition of the tin at the cathode.

It will thus be seen that most, if not all, tin electroplating baths, other than those using 45 metallic tin anodes, prepared with tin-bearing compounds become impotent with use due to impoverishment in metal content and the consequent accumulation of excess acid, alkali or salts thereof resulting from the 50 decomposition of the tin-bearing compounds present in the bath.

I have discovered that a tin-bearing com-

pound may be made which, though not appreciable soluble in water, is soluble in and combines with certain acids, such as hydrochloric acid; certain alkalies, such as sodium hydroxide; and with certain salts, such as sodium cyanide, when said acids, alkalies or salts are in aqueous solution. This tin-bearing compound does not, of itself, introduce 55 acid or alkali when used to form, or as a component of, certain tin electroplating baths, but it does introduce tin into these electroplating baths by reason of its composition.

By virtue of the property of this tin-bearing compound of dissolving in the aqueous solution of certain acids, such as hydrochloric acid, certain alkalies, such as sodium hydroxide and certain salts, such as sodium 70 cyanide, and combining therewith, it is suitable for preparing certain tin electroplating baths of a desired initial tin content, within the limits of its solubility, by the addition of this tin-bearing compound to baths containing definite known quantities of such acids, alkalies, or salts. This tin-bearing compound is also suitable for addition, either 75 in excess at the start or gradually during the progress of the electrodeposition, to certain tin electroplating baths wherein certain acids, such as hydrochloric acid, certain alkalies, such as sodium hydroxide and certain salts, such as sodium cyanide, are formed by the decomposition of the components of these 80 baths in the course of the electrolysis. Thus, this tin-bearing compound is suitable for addition to tin electroplating baths prepared from such tin-bearing compounds as an alkali metal stannate (sodium stannate), 85 wherein an alkali metal hydroxide, such as sodium hydroxide, is formed due to the decomposition of the alkali metal stannate by the removal of tin from the bath by electrodeposition.

Again, this tin-bearing compound is suitable for addition to tin electroplating baths prepared from such tin-bearing compounds as stannous chloride, wherein an acid, hydrochloric acid, is formed due to decomposition of the stannous chloride by the removal 90 of tin from the bath by electrodeposition.

A tin-bearing compound having the properties hereinbefore described may be pre-

pared by treating the aqueous solution of a stannate, such as sodium stannate, with a sufficient quantity of a suitable acid, acid salt or gas of acid character to neutralize, wholly or in part, the alkali of the stannate, thereby causing the formation within, and precipitation from, the solution of the tin bearing compound. The tin-bearing compound so formed may be separated from the surrounding solution by filtration, settling or other appropriate means and is then preferably washed with water to remove soluble admixed salts resulting from the neutralization, whole or partial, of the alkali of the stannate. The precipitate is not dried, since upon drying its solubility in such acids as hydrochloric acid, such alkalies as sodium hydroxide and such salts as sodium cyanide is lowered.

20 The tin-bearing compound, prepared as described, is practically neutral, in itself, and is only slightly soluble in water. It is, however, readily soluble in acids, such as hydrochloric acid, and in alkalies, such as 25 sodium hydroxide, even in dilute solution, and reacts with these acids and alkalies to form definite chemical compounds. Thus, with an acid, such as hydrochloric acid, a chloride of tin results, and with an alkali, such as sodium hydroxide, sodium stannate is formed. The soluble tin-bearing compound as prepared for use in the practice of this invention is a white, amorphous, semi-plastic mass, containing approximately 35 metallic tin and about 46% water.

The stannate solution from which the tin-bearing compound is made may be of any concentration, but is preferably used in an undersaturated condition. When an acid is 40 used as a precipitant, it may be diluted with water, say an equal volume; although the concentration of the acid is not of primary importance. The amount of acid to be added, however, is that which will be required 45 for neutralization of the alkali of the stannate, and this may be determined by analysis of a test portion of the stannate solution. The calculated amount of acid is then added to the stannate solution while the latter is kept agitated and preferably heated.

When an acid salt is used as the precipitant, such a salt is picked out as will break up under the application of heat and form a gas of acid character which in turn will react on the sodium stannate. The amount of such salt to be used will depend on the amount of acid gas which it will release under the application of heat and the quantity of sodium stannate present.

60 When an acid salt, such as sodium bicarbonate, is used as the precipitant, it is preferably dissolved in water, either hot or cold, and this solution is then added to the stannate solution. The intimate mixture of the two solutions, preferably by agitation, is

brought about and the sodium bicarbonate is decomposed by heating the mixed solutions. The decomposition of the sodium bicarbonate brought about by heating the solution causes the liberation of carbon dioxide which, combining with the alkali of the stannate, precipitates the tin-bearing compound. The amount of sodium bicarbonate required to treat a batch of stannate solution is based upon the carbon dioxide which will be liberated upon decomposing the bicarbonate by means of heat.

70 When a gas of acid character such as carbon dioxide, is used as the precipitant, the gas is brought into direct contact with the stannate solution. During the reaction with carbon dioxide, the stannate solution is preferably heated. The amount of carbon dioxide required to secure complete precipitation is determined by the quantity of alkali stannate present, since this reaction takes place only between the alkali of the stannate and the carbon dioxide. The quantity of carbon dioxide is determined by an analysis of a test portion of the stannate solution.

75 A specific example of a tin electroplating bath, in which the use of the tin-bearing compound, prepared as above described, represents an improvement over established practice, is that of a bath formed by solution of sodium stannate in water. As tin is electrodeposited from such a bath, sodium hydroxide is formed and, with continued electrolysis, accumulates in the bath to such an extent as to render the bath less efficient and ultimately unfit for further use, even though it may still contain a considerable amount of tin in the form of sodium stannate. A sufficient addition of the tin-bearing compound, prepared as herein described, to such an electroplating bath will restore the soluble tin content to normal and reduce the sodium hydroxide content, by causing the sodium hydroxide to react with the tin-bearing compound to form a fresh supply of water soluble sodium stannate. Any excess of the tin-bearing compound remains insoluble and inert until more sodium hydroxide is formed by electrolysis.

80 It is not feasible to use soluble tin anodes in an alkaline tin electroplating bath, since anode solution does not keep pace with cathode deposition. However, by the addition of the tin-bearing compound, prepared as herein described, using either tin or iron anodes, the tin content of the sodium stannate bath may be sustained and the excessive accumulation of free sodium hydroxide prevented.

85 In practice the tin-bearing compound, prepared as herein described, may be added in excess to the sodium stannate bath as the latter is made up and the compound remains

unaffected in the bath until electrodeposition begins. Then, as tin is deposited on the cathode and sodium hydroxide formed simultaneously in the bath, the tin-bearing compound dissolves in and reacts with the sodium hydroxide so formed to produce sodium stannate. The cycle of tin deposition, simultaneous sodium hydroxide formation and solution of the tin-bearing compound to form sodium stannate proceeds as described as long as the bath is operated.

The weight of the tin-bearing compound to be added to a sodium stannate bath should preferably be that which will supply sufficient metallic tin to the bath to compensate for the weight of tin which will be deposited from the bath during any given time. If desired, the tin-bearing compound may be added to a sodium stannate bath gradually during its use, so that an undissolved excess of the compound is present at all times.

In the sodium stannate bath, described above, the anodes may be formed of iron or other material of suitable shape and size and the cathode formed by the article or articles to be electroplated.

Besides the example given, where the tin-bearing compound is used with a sodium stannate bath already formed, a sodium stannate bath may be formed initially from the tin-bearing compound, by dissolving calculated amounts, based on its tin content, of the tin-bearing compound in sodium hydroxide or by the addition of an excess, i. e., more than will dissolve therein, to a calculated amount of sodium hydroxide, thus yielding a sodium stannate electroplating bath of any desired initial tin content, which may thereafter be sustained, during electrolysis, by keeping an undissolved excess of the tin-bearing compound present at all times.

Where the tin-electrolyte is stannous chloride in solution, the reaction during the electrodeposition of the tin results in the formation in the electrolyte of hydrochloric acid. The tin-bearing compound, prepared as herein described, may be added to this electrolyte in the same manner as hereinbefore described in connection with a sodium stannate electrolyte. The hydrochloric acid in the stannous chloride electrolyte reacts with the tin-bearing compound to form water soluble tin chloride, and thereby the tin content of the electrodeposition bath is maintained and excessive accumulation of hydrochloric acid prevented. If desired the tin electrolyte may be initially formed by the solution of the tin-bearing compound in hydrochloric acid.

The invention, while of particular advantage in electroplating tin, may be applied to any method of tin electrodeposition, such,

for example, as the production of pig-tin by electrolysis and subsequent smelting.

I claim:

1. The improvement in the electrodeposition of tin employing an appropriate electrolyte, which comprises supplying tin to the electrolyte by the introduction thereto of a compound of tin that is substantially insoluble in water but soluble in the products of the electrolysis forming in the electrolyte as electrodeposition proceeds. 75

2. The improvement in the electrodeposition of tin from an appropriate electrolyte, which comprises supplying tin to the electrolyte by the introduction thereto of a compound of tin that is substantially insoluble in water but soluble in the electrolyte as electrodeposition proceeds, said compound of tin of itself supplying no acid or alkali component when introduced into the electrolyte. 80

3. The improvement in the electrodeposition of tin from an appropriate electrolyte, which comprises supplying tin to the electrolyte by the gradually regulated introduction thereto of a compound of tin that is substantially insoluble in water but is soluble in and combines with the electrolyte and the products of electrolysis associated therewith. 85

4. The improvement in the electrodeposition of tin from an appropriate electrolyte, which comprises maintaining in the electrolyte an excess of a tin-bearing compound that is substantially insoluble in water but soluble in the electrolyte and the products of the electrolysis associated therewith. 95

5. The improvement in the electrodeposition of tin, which comprises preparing a tin-bearing electrolyte by dissolving in an appropriate solvent therefor a compound of tin that is substantially insoluble in water but soluble in solutions of hydrochloric acid, sodium hydroxide, and sodium cyanide. 100

6. The improvement in the electrodeposition of tin from an appropriate electrolyte, which comprises maintaining a fixed proportion of tin in solution in the electrolyte by adding thereto a tin-bearing compound which is substantially insoluble in water but chemically active to form a soluble tin salt with a product of the electrolysis associated with the electrolyte, said compound of tin of itself supplying no acid or alkali component to the electrolyte. 110

7. The improvement in the electrodeposition of tin from an electrolyte containing an alkali metal stannate, which comprises maintaining a fixed proportion of tin in solution in the electrolyte by adding thereto a tin-bearing compound substantially insoluble in water but soluble in the solution of alkali metal hydroxide formed in the electrolyte as tin is electrodeposited therefrom. 120

8. The improvement in the electrodeposi-

tion of tin, which comprises preparing a tin-bearing electrolyte by dissolving in an appropriate alkali metal hydroxide, such as sodium hydroxide, a compound of tin which is substantially insoluble in water but soluble in solutions of hydrochloric acid, sodium hydroxide, and sodium cyanide.

9. The improvement in the electrodeposition of tin from an appropriate electrolyte, 10 which comprises supplying tin to the electrolyte by the introduction thereto from time to time of a compound of tin that is substantially insoluble in water but soluble in the electrolyte and the products of electrolysis associated therewith, said compound

of tin supplying of itself no acid or alkali component to the electrolyte.

10. The improvement in the electrodeposition of tin from an appropriate electrolyte which comprises maintaining a substantially uniform concentration of tin in solution in the electrolyte by adding thereto from time to time a tin-bearing compound which is substantially insoluble in water but soluble in the electrolyte as electrodeposition proceeds, said compound of tin supplying of itself no acid or alkali component to the electrolyte. 20 25

In testimony whereof I affix my signature.  
HORACE RUSSELL McILHENNEY.